

## UNITED STATES PATENT OFFICE

1,996,567

## METHOD OF TREATING WOOD

Samuel D. Butterworth, Detroit, Mich., assignor  
of one-half to Josephine M. Butterworth, De-  
troit, Mich., and one-half to C. P. Gable, Gable,  
S. C.

No Drawing. Application November 7, 1930,  
Serial No. 494,166

4 Claims. (Cl. 99—12)

This invention has to do with the treatment of various kinds of woods and particularly the treatment of woods for use in an end grain manner. The invention is not to be limited to the use of 5 woods in this manner, but this is an advantageous manner of use of woods thus treated.

In my Patent #1,736,186 of November 19, 1929, there is described the method of treating certain kinds of wood to harden the wood and for bringing out coloring in the wood and grain effect. 10 The present invention relates to certain improved features in a method of this kind applicable to several different kinds of wood and in which the method is controllable in such manner that predetermined coloring or grain effects in the wood 15 may be produced. In addition to this the present method contemplates a sequence of steps such that the moisture content of the wood is not materially varied.

20 In general, the present method contemplates treating the wood with an oil which serves, among other things, to maintain the moisture content of the wood, and with an alkali which serves, at least in part, to bring out coloring and/or grain effect in the wood and which may also serve for hardening the wood. As examples of wood which can be thus treated woods of the pine family may be cited, such as for example, long leaf yellow pine, loblolly pine, and Rosemary 25 pine. Also cypress, particularly gulf red cypress; redwood, red cedar. Long leaf yellow pine is particularly adapted for treatment by the method as is gulf red cypress. These two woods are probably the ones to be preferred for the method, 30 although the other woods may be used.

The procedure contemplates utilizing wooden blocks cut in an end grain manner; that is to say, the grain runs in the direction of the short dimension of the block so that when the block 40 is laid on the floor, for example, the grain is disposed vertically. First the wood is properly dried as by means of a dry kiln to bring the moisture content to the desired point, and this may be done either before or after the wood is 45 cut into the blocks. These blocks of wood may be individually treated by the method, or they may be united to form a tile block consisting of several separate wooden blocks fitted and glued together.

50 The blocks of wood, or tile formed of several blocks, whichever happens to be preferred, may be first treated with an oil as by means of submerging the same in a bath. This bath may comprise a penetrating oil such as mineral spirits 55 which serves as a carrier for paraffin. The

quantity of mineral oil and spirits may vary, but about two pounds of paraffin to a gallon of mineral spirits is thought to be a satisfactory bath. Also, preferably, in this bath there is a small percentage, say for example, 5% of vegetable oil such as linseed or tung oil. This bath is kept fairly well heated, preferably about 150° F., and the block or blocks are submerged in the bath for a sufficient period to permit the penetrating oil to enter the pores of the wood 10 carrying with it, of course, the paraffin and vegetable oil. The length of this period is subject to variation and depends somewhat upon the particular wood employed, thickness of the blocks, etc., but about fifteen minutes for this 15 bath is thought to be sufficient.

Following this treatment, the wood is treated with an alkali. For this purpose the wood may be submerged in a bath of sodium silicate in which the alkali content is controlled as desired. An 20 example of such a bath may be 50% silicate of soda of normal specific gravity 42.5 Baumé and 50% of water. To this bath may be added alkali in sufficient quantity to effect the desired results, and for this purpose potassium hydroxide or sodium hydroxide may be used. This bath is also kept heated, say to 150° F. 25

In the first bath the mineral spirits penetrate the wood carrying into the wood the paraffin and linseed oil, and inasmuch as the mineral spirits 30 is volatile the inner pores and fiber of the wood are left with a content of paraffin which seals the wood as regards its moisture content. The linseed oil or tung oil crystallizes in the wood which effects a hardening of the wood and gives 35 it a hardened finish. The wood being treated may be withdrawn directly from the first oil bath and immediately immersed into the second alkali or water glass bath. Due to the fact that the wood has been previously treated with an oil 40 bath the same does not readily permit of penetration in the second bath. However, it has been discovered that by strengthening the alkali content of the second bath by the addition of an adequate amount of potash or caustic soda that 45 sufficient penetration into the wood for the purpose desired is effected. Color and grain effect of the wood is brought out by the action of the alkali and the extent to which the color and grain effect is produced may be controlled by the alkali 50 content of this bath. In other words, the greater the alkali content in the second bath, the greater the color producing effect. Sodium silicate in itself does not have great penetrating power in a block previously oil treated. But the penetrating 55

and coloring effect may be increased by the addition to the second bath of the potassium hydroxide or sodium hydroxide. The blocks may be left in this second bath sufficiently long to effect the desired result, this time may vary with different woods and other conditions, but about fifteen minutes for the second bath is thought to suffice. In any event the coloring may be controlled by the alkali content.

Another manner of proceeding is to form an emulsion of the substances of the first two baths, maintain it at the required temperature say, for example, at about 150° F., and treat the wood in the emulsion as by submerging the blocks. With this arrangement the penetration in the wood is slower so that the treatment is longer, although the total length of time required in the wood emulsion bath and in the separate baths is about the same. In other words, by maintaining the blocks of wood in the emulsion about thirty minutes will suffice.

The blocks may be treated by reversal of the sequence of the first two steps; that is to say, by first treating the blocks with the alkaline solution and later with the penetrating oil and paraffin. This, however, is not preferred especially for some uses of the wood because the moisture content may be varied due to the water getting into the wood in the first treatment. However, the alkali content of the first bath need not be so great in this case because the wood can be readily penetrated inasmuch as it is not first treated with oil, but even here the alkali content can be controlled in order to give predetermined color effects in the wood. If there is a substantial varying in the moisture content, the blocks of wood may swell up and not maintain their original size.

The sodium silicate also serves as a hardener for the wood. Where the wood is first treated with the sodium silicate the hardening effect may be substantially throughout the wood. When the wood is treated first with the oil the second treatment with the sodium silicate does not readily permit penetration into the wood. Accordingly, in this case the wood is hardened near its surface and the penetration thereof is sufficient to harden and color the wood to a sufficient depth so that it will withstand long usage and wear without losing its original color.

The linseed or tung oil may be omitted and the result accomplished satisfactory for many purposes, yet it is preferred that these, or other equivalent oils be used because the crystallization and hardening effect. The emulsion may be maintained in a substantially constant condition as by means of agitating the same.

Blocks or tile of wood thus treated may be used advantageously for end grain wooden flooring, and this is one of the most important uses although the wood may also be used in such

places as panel work, wainscoting, furniture or the like. In a floor the original color is maintained for a long period, and even where the blocks are first treated with the oil, paraffin, etc., the penetration in the succeeding alkali bath is sufficiently deep so that there is no danger of the flooring wearing away more than the penetration, and accordingly the hardened and colored surface is maintained so that there is substantially no show of wear.

I claim:

1. A method of treating long leaf yellow pine which comprises first treating the wood in a bath consisting of mineral spirits, paraffin carried by the mineral spirits, a quantity of linseed oil, then subjecting the wood to a bath of sodium silicate with an added alkaline constituent, and determining the amount of alkaline constituent to produce desired wood coloring.

2. A method of treating long leaf yellow pine which comprises first treating the wood in a bath consisting of mineral spirits, paraffin carried by the mineral spirits, a quantity of linseed oil, maintaining the bath at about 150° F., then subjecting the wood to a bath of sodium silicate with an added alkaline constituent, maintaining this bath at about 150° F., and determining the amount of alkaline constituent to produce desired wood coloring.

3. A method of fixing the moisture content, hardening and producing color in wood which comprises, first subjecting a piece of the wood to a heated bath of paraffin oil for a period sufficient for the paraffin oil to penetrate into the pores of the wood, then subjecting the said piece of wood to a heated alkaline bath of silicate of soda for a period sufficient for penetration of the alkali into the oil-carrying wood, and incorporating in said alkaline bath additional alkaline selected from the group which consists of potassium hydroxide or sodium hydroxide in such quantity as to give to the solution a requisite increase in penetrability into the wood to determine the coloring of the wood.

4. A method of fixing the moisture content, hardening and producing color in wood of the pine family which comprises, first subjecting a piece of the wood to a heated bath of paraffin oil for a period sufficient for the paraffin oil to penetrate into the pores of the wood, then subjecting the said piece of wood to a heated alkaline bath of silicate of soda for a period sufficient for penetration of the alkali into the oil-carrying wood, and incorporating in said alkaline bath additional alkaline selected from the group which consists of potassium hydroxide or sodium hydroxide in such quantity as to give to the solution a requisite increase in penetrability into the wood to determine the coloring of the wood.

SAMUEL D. BUTTERWORTH.